

July 15, 1924.

1,501,887

F. M. CRAPO

PROTECTED METAL AND PROCESS OF MAKING IT

Filed Dec. 10 1923



## UNITED STATES PATENT OFFICE.

FREDERICK M. CRAPO, OF MUNCIE, INDIANA, ASSIGNOR TO INDIANA STEEL & WIRE COMPANY, OF MUNCIE, INDIANA, A CORPORATION OF INDIANA.

## PROTECTED METAL AND PROCESS OF MAKING IT.

Application filed December 10, 1923. Serial No. 679,650.

To all whom it may concern:

Be it known that I, FREDERICK M. CRAPO, a citizen of the United States, residing at Muncie, in the county of Delaware and 5 State of Indiana, have invented a new and useful Protected Metal and Process of Making It, of which the following is a specification.

The primary object of my invention is 10 to improve the zinc-coating of iron and steel articles, and especially of iron and steel wire. More specifically, such primary object is to produce a zinc-coated article, especially iron or steel wire, the coating of 15 which will adhere firmly and will not peel or flake off even when subjected to sharp bends or twists, as for example upon wrapping a wire around its own diameter; and especially to accomplish all this effectively 20 with iron and low-carbon steel, with which such results can not be obtained by ordinary galvanizing.

It is a further object to get this improved 25 zinc-coating without adversely affecting the mechanical and electrical properties, such as tensile strength, elongation, and electrical resistivity.

A further object is to simplify, cheapen, and shorten the process of cleaning and 30 (or) annealing at any stage of the manufacture of iron and steel wire. This cleaning and (or) annealing may be used as a preparation for zinc-coating; or as a mere independent operation, without relation to 35 immediate zinc-coating, or to any zinc coating at all.

Still another object is to get a more satisfactory and lasting zinc-coating with a smaller amount of zinc.

40 In accomplishing these results, from the standpoint of zinc-coating, I pass the iron-base article, such as iron or low-carbon steel wire, advantageously after it has reached the gage at which it is to be coated and 45 preferably in a continuous operation in the case of wire, through a suitable surface-treating, advantageously in a bath, to prepare the surface for the application of the zinc-coating; and subsequently apply the 50 zinc-coating. I am not fully certain of the action of this surface-treating bath, but the

bath I have used with best success contains carbonizing material, such as a commercial cyanide mixture of any suitable proportions, maintained in molten condition 55 at a temperature advantageously between 1200° and 1300° F. I believe that this produces a superficial carbonizing action on the iron-base (or ferrous metal) body, and so produces a relatively high-carbon surface 60 condition. In any event, it has some action on the surface of the iron-base body so that when the coating of zinc is subsequently applied, as upon passing wire so treated through a bath of molten zinc, better adhesion of the coating is obtained, and the 65 coating has superior mechanical properties. It is my belief that the superior nature of the zinc coating which I obtain is accounted for primarily by the superficial carbonizing action before mentioned on the iron-base body, but it is also possible that it may be due to the improved condition of the 70 surface of the iron-base body or to these things in combination.

75 Further, by passing the wire through the bath referred to, I find that I obtain not only this surface-treating effect, probably a very thin surface carbonizing, but also obtain at least two additional and very valuable effects. In the first place, I find that I obtain a very effective annealing of the wire, following its various passages through the dies up to that point; so that it is possible completely to eliminate the usual annealing furnace which heretofore it has always been considered necessary to provide after the wire has been drawn down to a certain size. In the second place, I find that the bath of molten salts, in addition 80 to the surface-treating and the annealing effects, produces a most effective cleaning action; so that it is possible to eliminate or reduce the period of immersion in the acid bath or baths through which the annealed 85 wire is usually passed for cleaning just prior to entering the molten zinc, though I prefer to retain a short acid bath, or to provide a zinc chloride or other bath, just before the molten zinc, in order to get the 90 desired fluxing action.

95 Thus by the immersion of the iron-base

article in the aforesaid bath of molten salts I obtain a very effective chemical heat-treating, which has many advantages. By the term "chemical heat-treating", I mean the production in the iron-base (or ferrous-metal) body of both a permeative addition by chemical change and a heat-treatment; such for example as annealing and superficial carbonization, both of which occur in my bath of molten salts.

By avoiding or reducing the period of immersion in acid I practically eliminate loss of iron, for there is substantially no such loss in the chemical heat-treating. Further, I believe I avoid the occlusion of hydrogen in the surface of the iron-base body, such as occurs in acid treatment. This may contribute to the production of the surface condition which causes better adherence of the zinc coating when the latter is subsequently applied.

I prefer to treat the wire in this bath of molten salts after it has passed through all the dies necessary to reduce it to the desired gage, to get the cleaning and annealing action just prior to coating. However, so far as producing a non-peeling zinc coating is concerned, it is not essential that this surface treatment be at this point in the process. It may be at any earlier point in the process, though then it may be necessary to produce a second annealing and a cleaning just prior to zinc-coating, on account of intervening actions on the wire. When such a second annealing and cleaning is done, it may be either by passing the wire through a second and similar bath of molten salts, in accordance with my invention, or may be in the old way of passing the wire through an annealing furnace and then through an acid bath for cleaning. In other words, the surface effect which my bath of molten salts produces will follow the wire all the way through the series of dies or through any part thereof which may be desired.

In consequence, I have found it possible even to use this annealing and cleaning method on the original rods, of about one-quarter inch diameter, with which the wire-drawer starts in the manufacture of wire, and to obtain a most effective cleaning thereby. This makes it possible to eliminate the usual long and somewhat complicated method of cleaning rods prior to drawing. Further, by avoiding the acid pickling which forms part of the usual preparatory process, I largely eliminate the loss of iron and the occlusion of hydrogen already referred to, and also lessen or eliminate the tendency to become brittle. This preliminary cleaning and treatment in the bath of molten salts may be supplemented by one or more subsequent annealings and cleanings, whether in the same or some other manner; but whether or not there is any other sub-

sequent treatment by passing through a bath of molten salts, this preparatory treatment produces on the surface some effect, probably carbonizing, which persists throughout all the subsequent operations, and makes it possible to apply a better zinc coating, if desired, when the final gage has been reached.

Further, I have found that this treatment of the surface of the wire in the bath of molten salts produces some sort of preserving effect, even if there is no subsequent zinc-coating. In other words, a wire which has been treated by passing it through this bath of molten salts is found to be less susceptible to corrosion than the same wire which has not been so treated. The chemically heat-treated wire has a very dense and smooth surface, which even without further protection (as by zinc-coating) persists under adverse conditions.

In addition, this treatment of the surface of the wire by passing it through the bath of molten salts is found to have no detrimental effect on the electrical and mechanical properties of the wire; so that all the advantages of a low-carbon content are retained, and also there are added advantages.

In using this bath of molten salts, I have found it possible to vary the composition of the bath very greatly. I believe the bath should contain some carbonizing material, mixed with other things serving mainly as fillers or diluents. A most advantageous mixture which I have used contains 60% sodium cyanide, 20% sodium carbonate, and 20% sodium chloride. Further, the temperature of the bath may be varied quite considerably, and I have found the process very effective with temperatures ranging from about 1200° F. to about 1300° F.

The bath of molten salts may be covered with a thin layer of coke, if desired, to lessen exposure to the atmosphere and consequent heat loss due to radiation. This layer of coke also serves partly as a wipe for the wire as it leaves the bath, thus effecting a reduction in the loss of salts.

The bath is preferably so arranged that the wire remains in it only for a short time. No period of immersion which I have tried has proven too short, even down to 7 or 8 seconds; but I prefer an immersion of about 15 seconds, to obtain a more complete annealing and a desirable cleaning, as well as the desired surface treatment, and greater permissible tolerance in the period of immersion and the temperature of the bath.

In the accompanying drawings, I have illustrated apparatus for practicing my process and producing my improved product: Fig. 1 is a longitudinal sectional view showing diagrammatically an apparatus for surface-treating, annealing, and cleaning a wire by chemically heat-treating it after it has been drawn to the desired gage, and for zinc-

coating it following such chemical heat treating, all in continuous operation; and Fig. 2 is a longitudinal sectional view showing diagrammatically an apparatus for surface-treating and cleaning rods in a continuous process in preparation for wire-drawing.

Referring first to the apparatus shown in Fig. 1:—

The iron-base wire 10, of iron or low-carbon steel, is presumed to have been passed previously through the desired sizing dies, until it has reached the gage at which it is desired to zinc-coat it. Then it is passed through a tank 11, containing my bath of molten carbonizing salts; then, with sufficient interval for some cooling, through a bath 12 of water for removing any adhering salts; then through a fluxing bath 13 of any suitable flux, such as of hydrochloric acid or zinc chloride; and then through a bath 14 of molten zinc, in which the wire takes its zinc coating. From the zinc-coating bath 14, of molten zinc, the wire passes to the winding reel 15. All this is in a continuous process, 25 with the wire continuously moving in the direction of the arrows.

While the zinc coating may be applied in various ways, the way I prefer to apply it, especially to wire, is by passing the wire 30 through a bath of molten zinc. The zinc-coating bath 14 is advantageously maintained at about 840° F. to 900° F., in any convenient way; though that temperature may be varied at the judgment of the operator.

If desired, and usually it is desirable, a hot plate 16 may intervene between the fluxing bath 13 and the molten-zinc bath 14, so that the wire will be dry when it enters 40 the molten zinc.

The chemically heat-treating bath 11 contains the molten carbonizing salts 17, above referred to, preferably covered by a coke layer 18. These salts 17 are maintained at a 45 temperature somewhat above their melting point, advantageously between 1200° F. and 1300° F., as by a fire 19 below the bath 11. For carrying off fumes, a hood 20 is preferably provided over the bath 11. This 50 bath 11 serves to give the desired surface treatment, which it is the fundamental object of my invention to obtain. It also acts to produce the desired annealing and cleaning; so that the usual annealing furnace 55 may be dispensed with, and so that no acid bath is needed for cleaning, although a short acid bath 15 may be used for fluxing.

Referring now to the apparatus shown in Fig. 2:—

The rod 10' from which the series of drawing operations starts is passed through a tank 11', containing my bath of molten carbonizing salts; then through a bath 12' of water for removing any adhering salts; 65 and then to the winding reel 15'. All this

is in continuous operation. The molten salts 17' in the bath 11' produce a chemical heat-treatment on the rod 10', and effectively clean it; so that from the reel 15' the rod is ready to go to the drawing dies. The 70 salts 17' in the bath 11' are maintained in molten condition by a fire 19' below; may be covered by a layer of coke 18', if desired, though that is not necessary; and preferably have a hood 20' above them for carrying off 75 any fumes.

If desired, in order to lessen the time of immersion in the bath 11' of molten salts, the rods 10' may be passed through a bath 25 of molten lead just previous to entering 80 the bath 11'. The molten lead in the bath 25, when that bath is used, serves to heat the rod, so that less rise in temperature of the rod will be necessary in the bath of molten salts, and the period of immersion 85 in the molten salts may be reduced. The bath 25 of molten lead is thus merely a preliminary heating means for the rod or wire, and may be used as such preliminary whenever desired in practicing my invention; but 90 it is merely a convenient preliminary, and is not essential. It is not shown in Fig. 1.

I claim as my invention:—

1. A zinc-coated iron or steel article, comprising an iron-base body which is of relatively low carbon content in the interior but has a relatively high-carbon surface condition, and a coating of zinc upon and adhering to said high-carbon surface.

2. A zinc-coated iron or steel article, comprising a low-carbon iron-base body which has been treated in a bath of molten carbonizing salts, and a coating of zinc upon and adhering to the surface of such treated iron-base body.

3. A chemically heat-treated iron or low carbon steel article, and a zinc coating upon and adhering to such article.

4. Zinc-coated iron or steel wire, comprising an iron or steel core, and a zinc coating 110 thereupon and adhering thereto; the iron or steel core being of relatively low carbon content in the interior, but having a relatively high carbon content at the surface where it adjoins the zinc coating.

5. Zinc-coated iron or steel wire, comprising a low-carbon iron-base core which has been treated in a bath of molten carbonizing salts, and a coating of zinc upon and adhering to the surface of such treated 120 core.

6. Chemically heat-treated iron or low-carbon steel wire, and a zinc coating upon and adhering to such wire.

7. The process of zinc-coating an iron or 125 low-carbon steel article, which consists in immersing the article in a carbonizing bath of molten salts, and subsequently immersing it in a bath of molten zinc.

8. The process of zinc-coating an iron or 130

- 1 low-carbon steel article, which consists in immersing the article in a carbonizing bath of molten salts, and subsequently applying a zinc coating. 65
- 5 9. The process of zinc-coating an iron or low-carbon steel article, comprising increasing the carbon content at the surface of such article, and subsequently applying a zinc coating to such article. 70
- 10 10. The process set forth in claim 7, with the addition that the article is immersed in a fluxing material between its immersions in the two molten baths. 75
- 15 11. The process set forth in claim 7, with the addition that the article is washed and then treated with a flux between its immersion in the two molten baths. 80
- 20 12. The process of zinc-coating an iron or low-carbon steel article, comprising chemically heat-treating said article, including carbonizing the surface of said article, and subsequently zinc-coating such article. 85
- 25 13. The process of zinc-coating an iron or low-carbon steel article, comprising so chemically heat-treating the surface of said article, and subsequently zinc-coating such article. 90
- 30 14. The process of zinc-coating an iron or low-carbon steel article, comprising so chemically heat-treating the surface of said article that it promotes the bonding thereto of a zinc coating, and subsequently applying such zinc coating. 95
- 35 15. The process of zinc-coating an iron or steel article, comprising annealing and cleaning such article and producing a permeative addition by chemical change in the surface of such article in a single operation, and subsequently applying a zinc coating to such article. 100
- 40 16. The process of zinc-coating an iron or steel article of such composition that ordinary galvanizing thereof produces a coating which peels and cracks on bending or twisting, comprising chemically heat-treating such article to produce a surface-condition thereof, which on coating with zinc will take a substantially non-peeling coating; and subsequently applying such zinc coating. 105
- 45 17. The process of making zinc-coated iron or low-carbon steel wire, which consists in drawing the wire to a desired gage, subsequently passing it through a carbonizing bath of molten salts to produce a carbonizing treatment of the surface of the wire and also to produce a cleaning and annealing of the wire, and subsequently passing the wire through a bath of molten zinc. 110
- 50 18. The process of making zinc-coated iron or low-carbon steel wire, which consists in drawing the wire to a desired gage, subsequently passing it through a bath of molten salts to produce such a chemical heat-treatment of the surface of the wire that the adherence of a zinc coating to such surface will be increased, and to produce a cleaning and annealing of the wire, and subsequently passing the wire through a bath of molten zinc. 115
- 55 19. The process of making zinc-coated iron or low-carbon steel wire, which consists in drawing the wire to a desired gage and carbonizing the surface of the wire, and subsequently passing the wire through a bath of molten zinc. 120
- 60 20. The process of making zinc-coated iron or steel wire, comprising drawing the wire to a desired gage; and at any desired stage in the manufacture of the wire passing the wire through a molten bath of carbonizing salts to produce an annealing and a cleaning and also a superficial change in the wire; and subsequently both to the drawing operation and to the passage of the wire through the bath of molten salts passing such wire through a bath of molten zinc to apply thereon a zinc coating. 125
- 65 21. The process of making zinc-coated iron or steel wire, comprising drawing the wire to a desired gage; and at any desired stage in the manufacture of the wire chemically heat-treating the wire; and subsequently both to the drawing and the heat-treating operations applying a zinc coating to such wire. 130
- 70 22. The process set forth in claim 21, with the addition that the treating and zinc-coating operations are continuous. 135
- 75 23. The process of zinc-coating iron or steel wire, comprising producing such a chemically different surface-condition of the wire by permeative addition by passing it continuously through a bath of molten salts that it has greater adherence for a zinc coating subsequently applied, while maintaining the other parts of such wire than the surface thereof without substantial chemical change, and subsequently applying a zinc coating to such wire. 140
- 80 24. The process of zinc-coating iron or steel wire, comprising producing such a change in the surface of the wire by chemically heat-treating the wire that its surface has greater adherence for a zinc coating subsequently applied, while maintaining the other parts of such wire than the surface thereof without substantial chemical change, and subsequently applying a zinc coating to such wire. 145
- 85 25. The process of making a zinc-coated iron or steel article, comprising making an iron-base body with a relatively high carbon content at its surface and a relatively low carbon content in its interior, and applying a zinc coating to the surface of such iron-base body. 150
- 90 26. The process of making a zinc-coated iron or steel wire, comprising making an

iron-base wire with a relatively high carbon content at its surface and a relatively low carbon content in its interior, and applying a zinc coating to the surface of such 5 iron-base wire.

27. The process of zinc-coating an iron or low-carbon steel article, comprising chemically heat-treating said article in a hot liq-

uid medium, and subsequently zinc-coating said article. 10

In witness whereof, I have hereunto set my hand at Washington, D. C., this 10th day of December, A. D. one thousand nine hundred and twenty three.

FREDERICK M. CRAPO.